

# United States Patent [19]

Nemoto et al.

[11] 3,855,015

[45] Dec. 17, 1974

[54] **WORK ROLL FOR HOT ROLLING**

[75] Inventors: **Tadashi Nemoto**, Takahagi; **Kiyoshi Watanabe**, Hitachi; **Tadaaki Kobayashi**, Hitachi; **Joo Ishihara**, Hitachi; **Kenji Ono**, Tokyo; **Kazuhiro Sonomoto**, Kitakyushu, all of Japan

[73] Assignees: **Hitachi, Ltd.; Hitachi Metals, Ltd.**, Tokyo, Japan

[22] Filed: **May 4, 1972**

[21] Appl. No.: **250,186**

**Related U.S. Application Data**

[63] Continuation-in-part of Ser. No. 86,406, Nov. 3, 1970, abandoned.

[30] **Foreign Application Priority Data**

Nov. 4, 1969 Japan ..... 44-87559

[52] U.S. Cl. ..... 148/34, 29/196.1

[51] Int. Cl. ..... C04b 35/00, B32b 15/00

[58] Field of Search ..... 75/124, 126 E, 126 D; 148/34, 36; 29/196.1

[56]

**References Cited**

UNITED STATES PATENTS

|           |         |        |          |
|-----------|---------|--------|----------|
| 2,069,260 | 2/1937  | Merten | 75/126 E |
| 2,572,191 | 10/1951 | Payson | 75/126 E |
| 2,590,835 | 4/1952  | Kirkby | 75/126 E |
| 2,848,323 | 8/1958  | Harris | 75/126 D |

|           |         |          |          |
|-----------|---------|----------|----------|
| 2,983,601 | 5/1961  | Fletcher | 75/126 E |
| 3,201,232 | 8/1965  | Thier    | 75/126 D |
| 3,291,655 | 12/1966 | Gill     | 75/126 E |
| 3,409,966 | 11/1968 | Hilbush  | 29/196.1 |

Primary Examiner—Hyland Bizot

Attorney, Agent, or Firm—Craig & Antonelli

[57] **ABSTRACT**

A work roll for hot rolling comprising a body portion composed of a steel having a ferrite structure and having a yield strength at least 40 kg/mm<sup>2</sup>, improvement wherein substantially the whole surface of said body portion in the axial direction is provided with a weld metal having a high smoothed surface and having a thickness of 7 to 50 mm, said weld metal consisting essentially of 0.2 to 0.8 wt% of C, 4 to 10 wt% of Cr, 1 to 4 wt% of Mo, 0.5 to 5 wt% of V, 0.1 to 1.5 wt% of Si, 0.1 to 3 wt% of Mn, up to 0.5 wt% of Ni, up to 0.015 wt% of P, up to 0.015 wt% of S, at least one of 0.01 to 0.5 wt% of Ti and 0.05 to 1 wt% of Al, and the balance of substantially Fe, said components other than Ti and Al showing a hot crack sensitivity value of 2.7 or less when calculated according to the formula,

$C(P + S + Si/25 + Ni/30) / 3Mn + Cr + Mo + V \times 10^3$

and said weld metal having such a structure that carbide particles have been distributed in a martensite matrix.

**9 Claims, 6 Drawing Figures**



SHEET 1 OF 3

FIG. 1



FIG. 2



SHEET 2 OF 3

FIG. 3



FIG. 4



PATENTED DEC 17 1974

3,855,015

SHLET 3 OF 3

FIG. 5



FIG. 6



## WORK ROLL FOR HOT ROLLING

## CROSS-REFERENCE TO THE RELATED APPLICATION:

This is a continuation-in-part of our copending application, Ser. No. 86,406 filed on Nov. 3, 1970, now abandoned.

## BACKGROUND OF THE INVENTION

## 1. Field of the Invention

This invention relates to a work roll for hot rolling of such a construction that a weld metal which is excellent in rolling characteristics and low in weld crack sensitivity has been formed over the whole surface of an arbor material.

## 2. Description of the Prior Art

Hot rolling is an operation carried out by heating a metal or alloy to above the recrystallization temperature thereof to increase the metal or alloy in plasticity and passing the heated metal or alloy between rolls rotating at normal temperature or at an elevated temperature to shape the same into plates, rods or structural shapes, thereby destroying the cast structure of the metal or alloy to impart uniform and excellent properties thereto.

The rolls of a rolling machine are composed of a work roll which directly rolls and deforms a metal or alloy, and a back-up roll which reinforces the said work roll. In the rolling of a metal or alloy, the work roll is brought to the most severe state. It is well known that the work roller is easily worn out since it contacts with a material to be rolled which has been heated to a high temperature, tends to form cracks on the surface due to thermal fatigue failure since it is repeatedly subjected to thermal stress, and tends to be roughened on the surface since cracked portions formed on the roll surface are fallen off or fused. Accordingly, the material to be used for manufacture of the work roll should be high in resistance to the above-mentioned phenomena. In addition, the work roll is required to be high in strength and sufficient in toughness, since the ratio of reduction in hot rolling which is observed at the time when a material to be rolled is inserted between rolls is high and the work roll is liable to be bent. The wear resistance, hot cracking resistance and surface roughening resistance are indispensable matters for the work roll, and are generally called rolling characteristics.

In order to impart the rolling characteristics of a high level to the work roll, the material to be used for manufacture of the work roll should be increased in hardness as far as possible. On the other hand, however, the work roll is required to be high in tenacity as well. Since hardness and tenacity are in a relation contrary to each other, there is naturally a certain limit in imparting excellent rolling characteristics to one roll. For the above reasons, the work roll of the prior art has been manufactured by forming a high hardness weld metal on the surface of an arbor composed of a material high in tenacity. There are many and various weld metals usable for hard-facing, as regulated in ASTM 399-56T. In practice, however, weld metals to be applied to hot rolling work rolls and the like rolls which are required to be high in level of rolling characteristics should be not only high in hardness but also fine in grain size so as to minimize the propagation of hot cracks formed, and be free from pin-holes, which fre-

quently become causes for surface-roughening due to the falling-off of portions where the pin-holes have been formed. Accordingly, weld metal materials are also limited to specific materials.

5 As the result of extensive studies, the present inventors have found that as the weld metal to be formed on the surface of a body material for a work roll for hot rolling, a weld metal having a martensite structure which contains about 0.2 to 0.8 % by weight of C is 10 most preferable among those regulated in ASTM 399-56T. This weld metal, however, frequently formed many hot cracks when formed on the surface of a roll body by an automatic welding operation, which is ordinarily adopted for hardfacing of the roll body. Accordingly, the inventors have investigated the cause therefor to find that during the course of solidification of the weld metal from its molten state, such elements as C, P and S, which are marked in segregation tendency, are 15 further concentrated to the grain boundary when the weld metal is subjected to automatic welding operation, which requires a greater heat input and a longer solidification time, and the said elements separate from each other due to external and internal restriction forces at the concentrated portion to form cracks, and that such elements as Cr and Mn have actions to inhibit the weld metal from cracking even when the amount of C is left unchanged. The above findings coincide with the effects on hot crack sensitivity of various components of the high tensile alloy steel which was proposed 20 by F. J. Wilkinson et al. [see F. J. Wilkinson, C. L. M. Cottrel: British Welding Journal, 1958 (12), pages 557-562]. That is, they proposed the equation

$$H.C.S. = C(P + S + Si/25 + Ni/100)/3Mn + Cr + Mo + V \times 10^3$$

35 (wherein H.C.S. is an abbreviation for hot crack sensitivity), and clarified that according to tungsten inert gas shielded arc welding, as weld metal having an H.C.S. value of 4 or less is high in resistance to hot 40 cracking. The effects of various components used in the above-mentioned weld metal coincided with the results obtained by the present inventors. The present inventors applied to the above-mentioned equation the results of experiments on a weld metal containing 0.20 to 0.60 % by weight of C, 1 to 12 % by weight of Cr, and, in addition thereto, Si, Mn, Ni, Mo, V, etc. which 45 had been formed by submerged arc welding, to find that the relation between the presence of cracks and the H.C.S. value is as shown in FIG. 1, wherein the black points indicate an Ni-free weld metal. From FIG. 1, it appears that the absence of Ni in the weld metal has broadened the transition zone (H.C.S. value 1.2 to 2.1) with respect to the crack formation. Accordingly, 50 in case the weld hot crack sensitivity observed in an automatic welding operation is applied to the equation proposed by Wilkinson et al., there is a question in the Ni coefficient adopted in said equation. According to the experience of the present inventors, it is considered that said Ni coefficient is too small. In view of this, the inventors investigated the range of distribution of H.C.S values by varying the Ni coefficient to find that the Ni coefficient is adequately 1/30 and, in this case, the transition zone for crack formation can be limited 55 to such a narrow H.C.S. value range as from 1.6 to 1.8, as shown in FIG. 2.

60 However, the limitation that the modified H.C.S. value is less than 1.6 is extremely severe because in the

case of a work roll or the like, which is required to be particularly high in surface roughening resistance, it is desired that the content of C in the weld metal used is increased within a possible range. That is, even when judged sensibly, it may be said that in case the content of C in a weld metal is 0.5 % by weight for example, the weld metal cannot be inhibited from hot cracking unless the value of  $3\text{Mn} + \text{Cr} + \text{Mo} + \text{V}$  is increased to about 20 % by weight, and thus various problems occur in practice.

As the result of studies on such various restrictions as mentioned above, the present inventors have found that the limit of the modified H.C.S. value can be broadened to 2.7 by alloying a proper amount of Ti and/or Al with the weld metal material.

#### SUMMARY OF THE INVENTION

##### 1. Objects of the Invention

A principal object of the present invention is to provide a work roll for hot rolling of such a construction that a weld metal, which is extremely low in weld crack sensitivity and excellent in rolling characteristics, has been formed on the surface of an body material.

Another object of the invention is to provide a work roll for hot rolling of such a construction that a weld metal, which is greatly inhibited in weld hot cracking at the time of automatic welding operation, has been formed on the surface of an body material.

##### 2. Statement of the Invention

The work roll for hot rolling which is provided according to the present invention comprise a body portion composed of a steel having a ferrite structure and having a yield strength at least  $40 \text{ kg/mm}^2$ , improvement wherein substantially the whole surface of said body portion in the axial direction is provided with a weld metal having a high smoothed surface and having a thickness of 7 to 50 mm, said weld metal consisting essentially of 0.2 to 0.8 wt% of C, 4 to 10 wt% of Cr, 1 to 4 wt% of Mo, 0.5 to 5 wt% of V, 0.1 to 1.5 wt% of Si, 0.1 to 3 wt% of Mn, up to 0.5 wt% of Ni, up to 0.015 wt% of P, up to 0.015 wt% of S, at least one of 0.01 to 0.5 wt% of Ti and 0.05 to 1 wt% of Al, and the balance of substantially Fe, said components other than Ti and Al showing a hot crack sensitivity value of 2.7 or less when calculated according to the formula,

$$C(P + S + Si/25 + Ni/30)/3Mn + Cr + Mo + V \times 10^3$$

and said weld metal having such a structure that carbide particles have been distributed in a martensite matrix.

The work roll according to the present invention is such that on the surface of a body has been formed a weld metal which is excellent in rolling characteristics and which does not cause weld hot cracking, so that the body may have been made of any material so far as it can withstand the bending force applied at the time of rolling. According to many experiments, such body material is preferably a steel having a ferrite structure high in ductility and having a yield strength of at least  $40 \text{ kg/mm}^2$ .

If the body which contacts with a material to be rolled has no excellent and uniform rolling characteristics all over the surface, the two sides of the material to be rolled differ from each other in degree of deformation or the roll is locally damaged. Accordingly, the weld metal should be formed to a uniform thickness over the whole surface of the body.

In order to form a weld metal excellent in rolling characteristics, it is necessary to regulate the thickness of the weld metal. If the thickness of the weld metal formed is less than 7 mm, the weld metal cannot display high wear resistance, while if the thickness is more than 50 mm, the number of steps required for formation of the weld metal becomes larger to bring about economical disadvantages.

The weld metal formed according to the present invention displays excellent rolling characteristics, i.e., high hot cracking resistance, wear resistance and surface roughening resistance. Further, the weld metal has been so controlled in composition that the effect of hot cracking prevention due to the presence of Ti and/or Al can sufficiently be displayed. Even when subjected to automatic welding operation, therefore, the weld metal does not bring about any such weld hot cracking as to be argued in practice, so far as the modified H.C.S. value thereof is up to 2.7.

Among the constituents of the weld metal, Cr dissolves in a major proportion into the matrix at the time of quenching to improve the quenching property thereof. Further, Cr is effective for prevention of hot cracking as well. From the standpoint of the quenching property improvement, Cr is required to be used in an amount of at least 4 % by weight. If the amount exceeds 10 % by weight, however, an eutectic of  $\text{Cr}_7\text{C}_3$  is developed in the form of network, with the result that hot cracking tends to take place. Accordingly, the amount of Cr should be made less than 10 % by weight. In order to obtain a weld metal which scarcely brings about hot cracking and which is excellent in quenching property, the amount of Cr to be used is preferably 6 to 9 % by weight.

Mn is also effective for prevention of hot cracking, like Cr, but if the content of Mn exceeds 3 % by weight, the retained austenite formed in the tissue of the weld metal is stabilized to make it difficult to apply thereto such heat treatments as quench-hardening and temper-hardening. The amount of 0.1 % by weight is the minimum amount of Mn to display its effect. Preferable range of Mn content is from 1 to 2 % by weight. So far as the content of Mn is within the above-mentioned range, the retained austenite formed in a welded state can easily be converted into martensite by subsequent heat treatment, and the effect of hot cracking prevention can effectively be displayed.

Si improves the oxidation resistance of the weld metal, and this effect is displayed when Si is used in an amount of at least 0.1 % by weight. However, Si increases the modified H.C.S. value, and hence is preferably used in a smaller amount. The amount of 1.5 % by weight is the critical amount of Si to inhibit the modified H.C.S. value to less than 2.7.

V forms, at the time of welding, a cluster together with C (which means such a state that the particles of V have clustered around the C) in the weld metal in a molten state to prevent hot cracking and, after solidification, bonds to C in an amount of about one-fifth to one-fourth the weight of V to form a vanadium carbide, thereby contributing to the improvement in wear resistance of the roll. A part of the vanadium carbide dissolves in the matrix at the time of quenching, and deposits and hardens at the time of tempering to increase the high temperature hardness of the roll. If the amount of V is less than 0.5 % by weight, the amount of V which dissolves in the matrix becomes smaller to make

it difficult to expect secondary hardening. If the amount of V is more than 1.5 % by weight, there are brought about such drawbacks that the vanadium carbide distributes to the state of network to make the weld metal brittle, and that in case the amount of C in the weld metal is 0.2 to 0.3 % by weight, substantially all of the C is converted into a carbide to bring the matrix to a ferrite structure, with the result that fusion-adhesion of the roll comes to be brought about. In order to facilitate the occurrence of secondary hardening of the matrix and to finely distribute the vanadium carbide, the amount of V should be within the range from 0.8 to 1.3 % by weight.

Mo is also effective for prevention of hot cracking, like V, and a part of Mo forms an  $M_6C$  type carbide after solidification. In this case, the amount of C required is about one-twentieth the amount of Mo, so that the amount of Mo can be made larger. However, if the amount of Mo carbide becomes larger, an eutectic thereof segregates in a network state to the grain boundaries to bring about detrimental effects. According to the experiments carried out by the present inventors, the amount of Mo is preferably 1 to 4 % by weight, more preferably 3 to 4 % by weight.

When the amounts of Mo and V have been so decided as mentioned above, the amount of C required may also be decided accordingly. In case Mo and V are incorporated in larger amounts than those defined above, the tendency of development of a ferrite structure undesirably becomes high. In order to form carbides together with Mo and V and to dissolve a part of C into the matrix, the amount of C should be made 0.2 to 0.8 % by weight. If the amount of C is less than 0.2 % by weight, the resulting weld metal comes to have a quenching hardening of less than 450 in terms of Vickers hardness (Hv) and is greatly deteriorated in surface roughening resistance. In case the amount of C is more than 0.2 % by weight, the C, which has dissolved in the matrix at the time of quenching, is hardened to make it possible to attain excellent surface roughening resistance. The upper limit of the amount of C is greatly dominated by the amounts of P and S contained as impurities and the amount of Si contained as a deoxidizer. However, in the case of a weld metal material, which had been prepared in consideration of the modified H.C.S. value and which had been incorporated with Ti or Al, the upper limit in amount of C was 0.8 % by weight. In order to make the weld metal entirely free from any cracks, the amount of C is desirably made less than 0.6 % by weight.

Ni tends to develop dendrite and has great influence on the modified H.C.S. value, so that the amount thereof is preferably as small as possible, and should not exceed 0.5 % by weight in any event.

P and S segregate to the grain boundaries to greatly promote the formation of weld hot cracks, and hence should be minimized as far as possible. Permissible amounts of P and S contained in the weld metal are individually 0.015 % by weight. In case the amount of each of P and S is more than 0.015 % by weight, and in case the amount of C is large, the weld metal necessarily brings about hot cracking unless Mn, Cr, Mo and V are incorporated therein in large amounts.

In order to impart excellent rolling characteristics to a weld metal formed on the surface of a body, the weld metal should have a matrix structure, concretely a martensite matrix structure, to which the highest hardness

can be imparted. Such structure can be attained by cooling the metal kept at a temperature capable of forming an austenite. More preferably, however, the said heat treatment should be effected after tempering the weld metal at about 720°C. before it is cooled to less than 200°C., whereby the weld metal can be prevented from formation of cold cracks.

Among weld metals formed on the surfaces of bodies, a weld metal, which displays particularly excellent rolling characteristics and which does not cause weld hot cracking, is consisted of 0.2 to 0.6 wt % of C, 6 to 9 wt% of Cr, 3 to 4 wt% of Mo, 0.8 to 1.3 wt % of V, 0.1 to 1.5 wt% of Si, 1 to 2 wt% of Mn, at least one of 0.01 to 0.3 wt% of Ti and 0.2 to 0.5 wt% of Al, up to 0.5 wt% of Ni, up to 0.015 wt% of P, up to 0.015 wt% of S, and the balance of substantially Fe, said components other than Ti and Al having a hot crack sensitivity value of less than 2.6 when calculated according to the formula,

$$C(P + S + Si/25 + Ni/30)/3Mn + Cr + Mo + V \times 10^3$$
,  
and more restrictively, the weld metal contains no substantial Ni, and the hot crack sensitivity value thereof is less than 2.6 when calculated according to the formula,

$$C(P + S + Si/25)/3Mn + Cr + Mo + V \times 10^3$$

#### BRIEF DESCRIPTION OF THE DRAWINGS

In the accompanying drawings,  
FIG. 1 is a graph showing the relation between the H.C.S. value of a weld metal when calculated according to the formula proposed by Wilkinson et al. and the state of crack formation of the weld metal;

FIG. 2 is a graph showing the relation between the H.C.S value of a weld metal when calculated according to the modified formula proposed by the present inventors and the state of crack formation of the weld metal;

FIG. 3 is a slant view of the construction of a sample prepared in order to carry out hot cracking test;

FIG. 4 is a graph showing the relation between the amounts of alloying elements and the ratio of crack formation;

FIG. 5 is a slant view showing the shape of a hot finishing work roll which is an embodiment of the present invention; and

FIG. 6 is a graph showing the heat treatment temperatures of weld metals formed on the surfaces of bodies.

#### EXAMPLE

In order to investigate the influence of Al and Ti on weld hot cracking, a weld metal was evaluated in hot cracking sensitivity according to bar type cracking test. The test was carried out in the below-mentioned manner:

Two bar materials, which were individually 32 mm. in diameter and 300 mm. in length, were so arranged as shown in FIG. 3, and were combined with each other by welding the two at portions distanced by 50 mm. from both ends. Subsequently, a flux and powders of alloying elements were sprinkled over the uncombined portions and melted by application of high frequency, and the bar materials were welded with each other according to submerged arc welding using a wire which had been processed in diameter to 4 mm. After the welding, the weld metal was subjected to post-heat treatment at 700°C. without lowering the temperature to below the pre-heating temperature so as to prevent the weld metal from cold cracking.

The crack sensitivity of the weld metal was decided in such a manner that the bead-bearing surface of the weld metal was shaved off by 2 mm. in thickness to measure the length of crack formed, and the sensitivity was evaluated in terms of a cracking ratio calculated according to the formula,

in the weld metal became about 35 % of the content thereof in the wire, and the content of Cr in the weld metal became about 45 % of the content thereof in the wire and thus somewhat higher than the content of Mo or V, since more or less amount of Cr had been supplemented from the flux.

Table 3

| Chemical composition of a weld metal formed when only iron powder was sprinkled (wt%) |      |      |       |       |      |      |      |         |  |
|---------------------------------------------------------------------------------------|------|------|-------|-------|------|------|------|---------|--|
| C                                                                                     | Si   | Mn   | P     | S     | Cr   | Mo   | V    | Fe      |  |
| 0.28                                                                                  | 0.59 | 0.91 | 0.018 | 0.023 | 2.49 | 0.45 | 0.33 | Balance |  |

Cracking ratio (%) = Total length of crack/Total length of bead  $\times 100$

In order to compare the effects of Ti and Al on crack sensitivity with those of other elements, the same test as above was effected using Fe, Mo and Cr as alloying elements.

In FIG. 3, 2 represents restriction beads welded to both ends of the material 1 to be welded; 3 represents the sprinkled flux and alloying element powders; and 4 represents the welded beads.

The materials used in the test and the chemical compositions thereof were as set forth in Table 1.

FIG. 4 shows the relation between the amounts of alloying elements and the crack ratio. As seen in FIG. 4, Cr, Mo, Ti and Al are effective for the reduction of crack ratio, and the order thereof in effectiveness is Ti > Al > Mo > Cr.

When viewed only from the standpoint of crack prevention, Ti displays a marked effect even when used in such a slight amount as about 0.01 wt%; Al displays a considerable effect when used in an amount of about 0.04 wt%, and brings about only crater cracking when used in an amount of more than 0.05 wt%; Mo tends to increase the crack ratio when used in an amount of more than 4 to 5 % by weight; and Cr tends to linearly

Table 1

| Kind of material            | Chemical composition (wt%) |      |      |      |       |       |       |       |    |    |      |
|-----------------------------|----------------------------|------|------|------|-------|-------|-------|-------|----|----|------|
|                             | C                          | Si   | Mn   | V    | P     | S     | Cr    | Mo    | Ti | Al | Fe   |
| Materials to be welded      | 0.31                       | 0.35 | 0.81 | —    | 0.022 | 0.029 | 0.06  | —     | —  | —  | Bal. |
| Wire                        | 0.39                       | 0.99 | 0.42 | 0.92 | 0.017 | 0.005 | 5.00  | 1.28  | —  | —  | Bal. |
| Iron powder (200 mesh)      | 0.04                       | 0.36 | 0.73 | —    | 0.008 | 0.008 | —     | —     | —  | —  | Bal. |
| Cr powder (100-150 mesh)    | —                          | —    | —    | —    | 0.006 | 0.005 | Bal.  | —     | —  | —  | —    |
| Alloying elements           | —                          | —    | —    | —    | 0.051 | 0.320 | 70.02 | —     | —  | —  | Bal. |
| Fe-Mo powder (100-150 mesh) | —                          | —    | —    | —    | 0.008 | 0.020 | —     | 42.13 | —  | —  | Bal. |
| Fe-Ti powder (200 mesh)     | 0.08                       | 0.07 | 0.04 | —    | —     | —     | —     | —     | —  | —  | Bal. |
| Al powder (200 mesh)        | —                          | —    | —    | —    | —     | —     | —     | —     | —  | —  | 1.65 |

Welding conditions were as set forth in Table 2.

Table 2

| Welding method      | Submerged arc welding                                             |
|---------------------|-------------------------------------------------------------------|
| Flux                | Bonded flux for hard-facing, produced by Kawasaki Iron-Making Co. |
| Pre-heating         | 200-250°C.                                                        |
| Welding current     | 600 A                                                             |
| Arc voltage         | 30 V                                                              |
| Welding rate        | 35 cm/min.                                                        |
| Post-heat treatment | 700°C. $\times$ 1 hour                                            |
| Furnace cooling     | —                                                                 |

The alloying elements were made definite in volume by addition of iron powder in order to avoid non-uniformity in thickness of the resulting weld metals which would be encountered when the alloying elements were small in amount.

The chemical composition of a weld metal formed by sprinkling only iron powder was as set forth in Table 3. As seen in Table 3, the content of each of Mo and V

reduces the crack ratio with increasing amount thereof. However, it has been confirmed that when the amounts of Mo and Cr become more than 4 wt% and 10 wt%, respectively, an eutectic of carbides is formed to make the formation of heats cracks easy, so that it is desired that the said elements are added in amounts as large as possible within the ranges of critical values thereof.

Table 4 is an extraction of the results of welding using several ten kinds of welding wires prepared on the basis of the results of experiments mentioned above, and shows the crack sensitivities and Vickers hardnesses of weld metals prepared by forming according to submerged welding six layers of each weld metal material on a mild steel plate of 50 mm. in thickness, 200 mm. in width and 300 mm. in length, by use of a wire which was melted by application of high frequency and processed to 4 mm. in diameter.

The welding was effected under the conditions of a current of 600 A, an arc voltage of 28 V, and a welding rate of 40 cm/min. As the flux, there was used a mixture of a bonded flux for hard-facing which had been

produced by Kawasaki Iron-Making Co. and a bonded flux for high tensile strength steel which had been produced by Kobe Steel Works.

The presence or absence of cracks was examined by investigating the cross-section and surface of each weld metal, and the hardness of each welding was measured after quenching the weld metal from 1,000°C. at a cooling rate of about 300°C/hour.

vantageous to add Ti. In case Ti has been incorporated into a weld metal material, the Ti oxide formed acts as a nucleus for solidification to make greater the total area of the grain boundary, whereby the concentrations of P and S can be lowered. Individual actions of Ti and Al are such that Ti has a desulfurizing action, and Al has an action of forming a compound together with Si to remove the compound as a slag.

Table 4

| Chemical composition of weld metal (%) |      |      |       |      |      |       |      |       |       | Properties of weld metal |                 |                       |               |
|----------------------------------------|------|------|-------|------|------|-------|------|-------|-------|--------------------------|-----------------|-----------------------|---------------|
| C                                      | Si   | Mn   | Cr    | Mo   | V    | Ti    | Al   | P     | S     | Fe                       | Modified H.C.S. | Crack formation       | Hardness (Hv) |
| 0.40                                   | 0.81 | 1.10 | 7.56  | 1.22 | 1.22 | —     | —    | 0.009 | 0.011 | Bal.                     | 1.8             | Internal fine cks.    | 513           |
| 0.39                                   | 0.77 | 1.10 | 7.12  | 1.32 | 1.26 | 0.11  | —    |       |       | Bal.                     | 1.8             | No cks.               | 505           |
| 0.64                                   | 0.63 | 0.99 | 9.36  | 2.43 | 1.24 | 0.04  | —    |       |       | Bal.                     | 2.4             | do.                   | 640           |
| 0.66                                   | 0.62 | 1.24 | 8.35  | 1.37 | 1.22 | 0.18  | —    | 0.005 | 0.010 | Bal.                     | 2.7             | do.                   | 641           |
| 0.76                                   | 0.65 | 1.13 | 10.06 | 2.29 | 1.14 | 0.14  | —    | 0.010 | 0.009 | Bal.                     | 2.7             | Slight fine cks.      | 718           |
| 0.83                                   | 0.63 | 1.08 | 9.48  | 2.31 | 1.03 | 0.25  | —    |       |       | Bal.                     | 3.1             | Fine cks.             | 755           |
| 0.85                                   | 0.70 | 1.22 | 10.05 | 2.14 | 1.15 | 0.18  | —    |       |       | Bal.                     | 3.0             | Large cks. at surface | 754           |
| 0.33                                   | 0.68 | 0.94 | 6.30  | 1.33 | 1.20 | —     | 0.04 |       |       | Bal.                     | 1.7             | No cks.               | 466           |
| 0.51                                   | 0.85 | 1.31 | 7.54  | 1.28 | 1.05 | —     | 0.01 | 0.008 | 0.013 | Bal.                     | 2.2             | Int. cks.             | 544           |
| 0.50                                   | 0.59 | 1.06 | 7.88  | 1.34 | 1.00 | —     | 0.52 |       |       | Bal.                     | 2.2             | No cks.               | 530           |
| 0.65                                   | 0.71 | 1.10 | 8.84  | 2.25 | 1.21 | —     | 0.43 |       |       | Bal.                     | 2.5             | No cks.               | 612           |
| 0.78                                   | 0.74 | 1.29 | 9.95  | 2.31 | 1.11 | —     | 0.50 |       |       | Bal.                     | 2.6             | Slight fine cks.      | 628           |
| 0.78                                   | 0.66 | 1.28 | 10.03 | 2.20 | 1.18 | —     | 0.96 | 0.005 | 0.019 | Bal.                     | 2.7             | do.                   | 501           |
| 0.72                                   | 0.69 | 1.28 | 9.33  | 2.09 | 1.26 | —     | 1.10 |       |       | Bal.                     | 2.6             | No cks.               | 438           |
| 0.61                                   | 0.68 | 1.14 | 9.08  | 2.05 | 1.27 | Ti+Al | 0.32 | 0.005 | 0.014 | Bal.                     | 2.3             | No cks.               | 609           |
| 0.55                                   | 0.72 | 1.19 | 7.09  | 1.31 | 1.24 |       | 0.28 |       |       | Bal.                     | 2.5             | do.                   | 583           |

As the result, it was confirmed that when Ti had been incorporated, the weld metal containing 0.66 wt% of C and having a modified H.C.S. value of 2.7 was completely prevented from cracking, and the weld metal containing 0.76 wt% of C and having a modified H.C.S. value of 2.7 formed slight cracks, but the degree of cracking was entirely negligible depending on the application purpose of the resulting work roll. In the latter weld metal, the amount of Cr is 10.06 wt% and thus is slightly excess of 10 wt%, which is the critical value of Cr. However, such a slight excess amount of Cr is involved in the scope of the present invention because no change is seen in the effectiveness of Cr.

When the amount of C exceeded 0.8 wt% and the modified H.C.S. value became 3 or more, the weld metal could not sufficiently be prevented from cracking in case the contents of Cr, Mo and V are within the aforesaid ranges.

The incorporation of Al resulted in no effectiveness unless the amount thereof was made somewhat larger than in the case of Ti. Further, when the alloying amount of Al exceeded 1 wt%, the weld metal became less than 450 Hv in hardness and was difficult for application to hot rolling work roll. When both Ti and Al were incorporated, the same effect of cracking prevention as above was observed as well.

Thus, so far as the amount of C is less than 0.8 wt%, it has become possible to elevate the upper limit of the modified H.C.S. value to 2.7 by incorporation of proper amounts of Ti and/or Al.

Both Ti and Al have deoxidizing and denitrifying actions to reduce the amounts of oxygen and nitrogen contained in the resulting weld metal and have actions to make crystal grains finer.

Ti is stronger in the above-mentioned actions, so that in case either one of Ti and Al is to be added, it is ad-

As is clear from FIG. 4 and Table 4, Ti is markedly effective even when used in a minute amount, but even if Ti is incorporated in an excessively large amount, it merely serves to form a carbide. For prevention of hot cracking, therefore, the amount of Ti to be incorporated should be limited to less than 0.5 wt%. Particularly excellent effect of Ti for the prevention of hot cracking is displayed when it is incorporated in an amount of 0.01 to 0.3 wt%. If the alloying amount of Al is less than 0.05 wt%, no substantial effect can be attained. According to Table 4, even the weld metal incorporated with 0.04 wt% of Al did not cause hot cracking. This is considered ascribable to the point that the weld metal was reduced in content of C to lower the modified H.C.S. value to 1.7, whereby such favorable result could be brought about. (This is judged from the fact that the weld metal containing 0.01 wt% of Al and having a modified H.C.S. value of 2.2 caused internal cracking.) When the content of Al exceeds 0.05 wt%, the cracking ratio quickly lowers, as is clear from FIG. 4, so that it is judged that the minimum amount of Al required is 0.05 wt%. However, if Al is incorporated in an excessively large amount, it dissolves in the matrix to promote the formation of ferrite, and lowers the hardness of the weld metal to bring about a cause for fusion-adhesion of the resulting work roll. Thus, the upper limit of Al amount is 1 wt%. In order to attain a high hardness without causing hot cracking, Al is preferably incorporated in an amount of 0.2 to 0.5 wt%.

The present inventors further attempted the incorporation of Zr. In this case, however, the effect of cracking prevention was not sufficient.

As an embodiment of the present invention, a work roll for hot finishing was produced. This roll had such a shape as shown in FIG. 5, and was composed of an body 10, a journal 11 which had been bonded to the

body, and a weld metal 12 formed on the surface of the body. The total length of the roll was 2,300 mm., the diameter of the body was 300 mm., the weld metal of 40 mm. in thickness had been formed over the whole surface of the body, and the surface of the weld metal had been mechanically polished to high smoothness. The body and journal were individually composed of 0.24 wt% of C, 0.32 wt% of Si, 0.78 wt% of Mn, 0.024 wt% of P, 0.021 wt% of S and the balance of Fe. The weld metal was composed of 0.41 wt% of C, 0.85 wt% of Si, 1.31 wt% of Mn, 0.011 wt% of P, 0.015 wt% of S, 5.01 wt% of Cr, 1.43 wt% of Mo, 0.98 wt% of V, 0.06 wt% of Ti and the balance of Fe, and had a modified H.C.S. value of 2.2.

The formation of the weld metal on the surface of the body was carried out in such a manner that according to submerged arc welding a wire of 4 mm. in diameter, which was composed of 0.59 wt% of C, 0.18 wt% of Si, 0.30 wt% of Mn, 0.008 wt% of P, 0.021 wt% of S, 5.33 wt% of Cr, 1.48 wt% of Mo, 1.10 wt% of V, 0.21 wt% of Ti and the balance of Fe, was spirally welded around the body, while rotating the body, under the conditions of a welding current of 600 A, an arc voltage of 30 V and a welding rate of 35 cm/min. As the flux was used a 4:1 mixture of a flux composed of 16 wt% of  $\text{SiO}_2$ , 16 wt% of  $\text{Al}_2\text{O}_3$ , 21 wt% of  $\text{CaO}$ , 31 wt% of  $\text{MnO}$ , 7 wt% of  $\text{CaF}_2$ , 4 wt% of  $\text{Fe}_2\text{O}_3$  and 3 wt% of  $\text{Na}_2\text{O}_3$ , and a flux composed of 20 wt% of  $\text{CaCO}_3$ , 40 wt% of  $\text{CaF}_2$ , 15 wt% of Mn and 25 wt% of Fe-Ti. At the time of welding, the body surface was preheated to 200° to 250°C. and, during the welding, the substratum temperature was maintained at 200° to 300°C. After the welding, the weld metal was immediately heated to 720°C., maintained at said temperature for 2 hours, and then cooled in a furnace.

The thus produced work roll was mechanically processed and then subjected to dye penetrant inspection test to examine the presence or absence of weld defects, but the presence of hot cracks and pin-holes was not observed at all.

The heat treatment characteristics of the above-mentioned weld metal were examined by use of a separately prepared test piece to find that even when cooled at a rate of 300°C/hr from 1,000°C., the weld metal could be sufficiently quenched, and that the weld metal was satisfactory also in hardness after tempering, showing a Hv value of about 500, as seen in FIG. 7.

The work roll was heated at 1,000°C. for 1 hour, cooled to room temperature at a rate of 300°C/hr, again heated to 500°C., maintained at said temperature for 2 hours, and then air-cooled. The weld metal of the work roll thus obtained had such a structure that fine carbide particles had been distributed in the tempered martensite matrix.

In order to investigate the extent in surface roughening resistance and wear resistance of the thus produced work roll, test pieces identical in composition with the weld metal of the roll were prepared and subjected to individual tests after definite heat treatments. The surface roughening resistance test was carried out in such a manner that a ring-shaped test piece was heated in steam at 570°C. for 1.5 hours to form a black oxide film on the surface thereof, and then contacted under a contact pressure of 50 kg. with another ring-shaped test piece composed of 0.37 wt% of C, 0.18 wt% of Si, 0.40 wt% of Mn, 0.024 wt% of P, 0.029 wt% of S, 5.10 wt% of Cr, 1.20 wt% of Mo, 0.90 wt% of V and the balance

of Fe. Thereafter, the black oxide film-bearing test piece was rotated at 500 r.p.m. and the other test piece was rotated in the same direction at a rate of 4 % slower than 500 r.p.m. After the lapse of 30 minutes, the rotation was ceased, and the degree of peeling of the black oxide film was measured. As the result, the thickness of the black oxide film became about one-half the thickness before the test, and the peeling degree was about 50 %.

The above-mentioned test was applied also to a cast steel composed of 1.60 wt% of C, 0.50 wt% of Si, 0.30 wt% of Mn, 0.50 wt% of Ni, 0.95 wt% of Cr, 0.29 wt% of Mo and the balance of Fe which was well known as a material excellent in surface roughening resistance. In this case, the thickness of the black oxide film became about three-tenths the thickness before the test, and the peeling degree was about 70 %.

The wear resistance test was effected in such a manner that a ring-shaped test piece was contacted under a contact pressure of 40 kg. with another test piece composed of 0.29 wt% of C, 0.20 wt% of Si, 0.70 wt% of Mn, 0.029 wt% of P, 0.03 wt% of S and the balance of Fe. Thereafter, the former test piece was rotated at 500 r.p.m. at room temperature, and the latter test piece was rotated in the same direction at a rate of 10 % slower than 500 r.p.m. After the former test piece had rotated  $6 \times 10^4$  times, the rotation was discontinued and the weight loss of the test piece due to wearing was measured. As the result, the weight loss due to wearing of the test piece was 1 g.

The above-mentioned test was applied also to a cast steel composed of 1.02 wt% of C, 0.58 wt% of Si, 0.72 wt% of Mn, 0.32 wt% of Ni, 0.90 wt% of Cr, 0.27 wt% of Mo and the balance of Fe, and to a forged steel composed of 0.85 wt% of C, 0.35 wt% of Si, 0.45 wt% of Mn, 2.2 wt% of Cr, 0.25 wt% of Mo and the balance of Fe. In these cases, the weight loss of the former steel was 3.75 g., and that of the latter steel was 1.8 g.

#### What is claimed is:

1. A work roll for use in hot rolling of a steel comprising a body portion composed of a steel having a ferrite structure and having a yield strength of at least 40  $\text{Kg/mm}^2$ , and a working layer of weld metal welded by submerged arc welding on the surface of said body portion, said working layer having a smooth surface and having a thickness of 7 to 50 mm, said working layer consisting essentially of 0.2 to 0.8 wt% of C, 4 to 10 wt% of Cr, 1 to 4 wt% of Mo, 0.5 to 5 wt% of V, 0.1 to 1.5 wt% of Si, 0.1 to 3 wt% of Mn, up to 0.5 wt% of Ni, up to 0.015 wt% of P, up to 0.015 wt% of S, at least one of 0.01 to 0.5 wt% of Ti and 0.05 to 1 wt% of Al, and the balance of substantially Fe, said components other than Ti and Al showing a hot crack sensitivity value of 2.7 or less when calculated according to the formula,

$$C(P+S+Si/25+Ni/30)/3Mn+Cr+Mo+V \times 10^3$$

and said working layer having a structure comprising carbide particles distributed in a martensite matrix produced by maintaining said working layer at a temperature at which it is capable of forming an austenite structure and thereafter cooling said working layer.

2. A work roll for use in hot rolling of a steel comprising a body portion composed of a steel having a ferrite structure and having a yield strength of at least 40  $\text{Kg/mm}^2$ , and a working layer of weld metal welded by submerged arc welding on the surface of said body

portion, said working layer having a smooth surface and having a thickness of 7 to 50 mm, said weld metal consisting essentially of 0.2 to 0.6 wt% of C, 6 to 9 wt% of Cr, 3 to 4 wt% of Mo, 0.8 to 1.3 wt% of V, 0.1 to 1.5 wt% of Si, 1 to 2 wt% of Mn, at least one of 0.01 to 0.3 wt% of Ti and 0.2 to 0.5 wt% of Al, up to 0.5 wt% of Ni, up to 0.015 wt% of P, up to 0.015 wt% of S and the balance of substantially Fe, said components other than Ti and Al showing a hot crack sensitivity value of 2.7 or less when calculated according to the formula,

$$C(P+S+Si/25+Ni/30)/3Mn+Cr+Mo+V \times 10^3$$

said working layer having a structure comprising carbide particles distributed in a martensite matrix produced by maintaining said working layer at a temperature at which it is capable of forming an austenite structure and thereafter cooling said working layer.

3. A work roll for use in hot rolling of a steel comprising a body portion composed of a steel having a ferrite structure and having a yield strength of at least 40 Kg/mm<sup>2</sup>, and a working layer of weld metal welded by submerged arc welding on the surface of said body portion, said working layer having a smooth surface and having a thickness of 7 to 50 mm, said weld metal consisting essentially of 0.2 to 0.6 wt% of C, 6 to 9 wt% of Cr, 3 to 4 wt% of Mo, 0.8 to 1.3 wt% of V, 0.1 to 1.5 wt% of Si, 1 to 2 wt% of Mn, at least one of 0.01 to 0.3 wt% of Ti and 0.2 to 0.5 wt% of Al, up to 0.015 wt% of P, up to 0.015 wt% of S and the balance of substantially Fe, said components other than Ti and Al showing a hot crack sensitivity value of 2.7 or less when calculated according to the formula

$$C(P+S+Si/25+Ni/30)/3Mn+Cr+Mo+V \times 10^3$$

and said working layer having a structure comprising carbide particles distributed in a martensite matrix produced by maintaining said working layer at a temperature at which it is capable of forming an austenite structure and thereafter cooling said working layer.

4. A work roll for use in hot rolling of a steel comprising a body portion composed of a steel having a ferrite structure and having a yield strength at least 40 Kg/mm<sup>2</sup>, and a working layer of weld metal welded by submerged arc welding on the surface of said body portion, said working layer having a high smoothed surface and having a thickness of 7 to 50 mm, said weld metal consisting essentially of 0.2 to 0.6 wt% of C, 6 to 9 wt% of Cr, 3 to 4 wt% of Mo, 0.8 to 1.3 wt% of V, 0.1 to 1.5 wt% of Si, 1 to 2 wt% of Mn, 0.01 to 0.3 wt% of Ti, up to 0.015 wt% of P, up to 0.015 wt% of S and the balance of substantially Fe, said components other than Ti showing a hot crack sensitivity value of 2.6 or less when calculated according to the formula,

$$C(P+S+Si/25)/3Mn+Cr+Mo+V \times 10^3$$

and said working layer having a structure comprising carbide particles distributed in a martensite matrix produced by maintaining said working layer at a temperature at which it is capable of forming an austenite structure and thereafter cooling said working layer.

5. A work roll for hot rolling a cast structure of a metal or alloy in which the cast structure is heated to above its recrystallization temperature to increase its plasticity and the cast structure is passed between said work roll and a back-up roll in order to shape said cast structure into plates, rods or other structural shapes, said work roll comprising:

a body portion composed of a mild steel or a steel having about 0.24 wt% C, the steel of said body portion having a ferritic structure and having a yield strength of at least 40 Kg/mm<sup>2</sup>, and a working layer of a weld metal welded by submerged arc welding on the surface of said body portion, said working layer having a smooth surface and having a thickness of 7 to 50 mm, said working layer consisting essentially of 0.2 to 0.8 wt% of C, 4 to 10 wt% of Cr, 1 to 4 wt% of Mo, 0.8 to 1.3 wt% of V, 0.1 to 1.5 wt% of Si, 1 to 2 wt% of Mn, at least one of 0.01 to 1.3 wt% of Ti and 0.2 to 0.5 wt% of Al, up to 0.5 wt% of Ni, up to 0.015 wt% of P, up to 0.015 wt% of S and the balance of substantially Fe, said components other than Ti and Al showing a hot crack sensitivity value of 2.7 or less when calculated according to the formula,

$$C(P+S+Si/25+Ni/30)/3Mn+Cr+Mo+V \times 10^3$$

and said working layer having a structure comprising carbide particles distributed in a martensite matrix produced by maintaining said working layer at a temperature at which it is capable of forming an austenite structure and thereafter cooling said working layer.

6. A work roll according to claim 5, wherein said body portion is composed of a mild steel.

7. A work roll according to claim 5, wherein said body portion is composed of a steel consisting essentially of about 0.24 wt% C, about 0.32 wt% Si, about 0.78 wt% Mn, about 0.024 wt% P, about 0.02 wt% S and the balance Fe.

8. A work roll according to claim 5, wherein the structure of said working layer is produced by heating said weld metal to a temperature of about 720° C and thereafter cooling.

9. The work roll of claim 8, wherein said weld metal is maintained at a temperature of about 720° C for about 2 hours before being cooled.

\* \* \* \* \*